

June 5, 1934.

S. RUBEN

1,961,509

ELECTRIC LAMP AND FILAMENT THEREFOR

Filed Nov. 29, 1929

Fig. 1.



Fig. 2.



INVENTOR

SAMUEL RUBEN

BY

*Chester W. Brantley*  
ATTORNEY

## UNITED STATES PATENT OFFICE

1,961,509

ELECTRIC LAMP AND FILAMENT  
THEREFORSamuel Ruben, New York, N. Y., assignor to  
Sirian Lamp Company, Newark, N. J., a cor-  
poration of Delaware

Application November 29, 1929, Serial No. 410,310

5 Claims. (Cl. 176—131)

This invention relates to incandescent lamps, filaments therefor, and process and apparatus for making the same.

More specifically, the invention relates to a new 5 type of electric lamp suitable for use in house lighting, automobile lighting, projector illumination and various other types of illuminating devices. The invention also pertains to a coated filament adapted to be heated by the passage of 10 electricity therethrough.

Among the objects of the invention is to provide a filament adapted for use in lamps and other means of light projection and illumination, having a core or base of refractory material such 15 as tungsten on which is placed a coating having such properties as to increase the light and life efficiency of the filament.

Another object is to provide a coated filament in an electric lamp, the coating being secured to 20 the core substance by means which secure a minimum loss of heat efficiency while the filament is in use for illumination.

Still another object of the invention is to provide a coated filament having a bonding agent 25 capable of resisting the high temperatures of an electric lamp filament to a degree approximately equivalent to that of the core and coating substances.

Another object of the invention is the provision 30 of a coated type filament for an electric lamp wherein vaporization, especially in the presence of gas pressure, is noticeably reduced.

Additional objects of the invention reside in the improved apparatus and processes which result 35 in greater efficiency of operation for a lamp made in accordance with the detailed specification hereinafter set forth, and in accordance with the accompanying drawing, wherein

Fig. 1 is a view of an ordinary type of incandescent lamp of the filamentary type; and

Fig. 2 is an enlarged sectional view through the filament.

The numeral 10 designates a glass envelope of ordinary type electric incandescent lamp, to one 45 end of which is secured a threaded base element 11. Within the envelope 10 and mounted in the base is the stem 12 which is extended into the filament support 14. The spider 15 is mounted on the support rod 14 and consists in a number of 50 oppositely extending rods terminating in hooks 19. A similar spider 20 is mounted adjacent the base of the support rod above the stem at 21, the rods of this spider 20 also terminating in hooks 22. The filament 13 is wound over the 55 spider hooks, as shown in Fig. 1, and the ends

thereof secured to the electric terminals 23 and 24.

In Fig. 2 is shown a cross-sectional view of the filament greatly enlarged to bring out the relative position of the layers or coatings which form the essence of this invention. A filament of an elementary metal, such as tungsten or tantalum, is well known. These elements have been eminently satisfactory as filaments for electric lamps because of their refractory characteristics and fairly low rate of vaporization, particularly when 60 employed in conjunction with gas within the lamp envelope. Theoretically, the tungsten filament, for example, may be improved by the utilization of a coating thereon which would have light radiating properties more selective to visible radiations than tungsten alone. Certain materials, such as combinations of thorium and cerium, as used in the Welsbach mantle, are illustrative of this type of illumination. Another field of improvement in a tungsten lamp would be toward 65 the utilization of a coating which would decrease the vapor pressure. Such improvements I have, in a measure, accomplished in the present invention, which utilizes a core material 16, made of tungsten or similar refractory metal such as 70 tantalum on which I have provided an intermediate coating of beryllium aluminosilicate and an outer surface layer of beryllium oxide, these two 75 coatings being intimately associated with each other and bound together to form an integral filament.

In determining the constituent materials of the coatings, I found that for insulators the lower the atomic number of the metal elements entering into the insulator the higher the specific 80 resistance thereof and the higher the temperature at which the insulating qualities are maintained. In other words, compounds of barium, calcium, 85 cadmium, strontium and zinc lose their insulating qualities and become conductive at relatively 90 low temperatures, while compounds of boron, magnesium, aluminum, silicon and beryllium have insulative characteristics at much higher 95 temperatures, such temperatures varying substantially inversely in each group as the atomic 100 numbers, beryllium and magnesium having the lowest numbers, and the compounds having the highest specific resistance, and these may be heated to extremely high temperatures without decomposing or losing their insulating qualities. Beryllium is better in this respect than magnesium, and has desirable properties as an illuminant, and for use with filaments of vacuum tubes therefore, where high temperatures and selective 105 illumination are desirable, I prefer to use com- 110

pounds of beryllium, although I do not wish to limit myself to this particular metal.

To attain the objects of the invention I have found it necessary to provide a graded coating 5 with a base layer next to the core wire which will fuse to the core at temperatures very much higher than normal operating temperatures, which will therefore act as a bonding agent between the core and an outer layer, with which outer layer it is 10 adapted to have a slight chemical reaction so as to closely combine the two layers together. This outer layer must be highly refractory at the maximum operating temperatures.

The inner or base layer of the coating may be 15 made by mixing finely ground beryllium aluminosilicate ( $3\text{BeO},\text{Al}_2\text{O}_3,6\text{SiO}_2$ ) with ammonium borate ( $\text{NH}_4\text{B}_2\text{O}_4$ ) in the proportion by weight of three of beryllium aluminosilicate to one of ammonium borate with enough water to give proper consistency. The beryllium aluminosilicate should 20 be ground fine enough to fall through a size 250 screen mesh; that is, a screen mesh having 250 apertures to the inch. This mixture is coated upon the core wire which, as previously stated, 25 may be of tungsten or any other desirable material having analogous or similar refractory and other properties, making it suitable for use in an electric lamp, and a current of about one and one-half (1.5) amperes is then passed through the 30 wire to heat it and dry the coating in place. I have found it preferable to apply two coats of this material to form the inner layer of the insulating coating, although more layers may be added if found desirable. Two coats make the 35 thickness approximately 0.01 of a millimeter.

The outer layer is preferably made of beryllium oxide ( $\text{Be}_2\text{O}_3$ ). The coating material for this oxide is prepared by grinding the oxide in a ball mill with twenty-five percent (25%) by weight 40 of ammonium borate, and enough distilled water to give the desired consistency. The mixture is then applied to the filament carrying the intermediate coating of beryllium silicate. This application is made while the filament is cold and the 45 coated filament is then heated to about 500° C. at which temperature the ammonium borate decomposes, forming ammonia gas, water vapor and boric oxide. At least five successive coatings of beryllium oxide material should be applied. 50 The successive heatings through the coating process also cause a partial sintering of the coating material.

The wire thus provided with its insulating coating may be handled and bent and welded in position 55 in a lamp or other appliance in which the wire is to be used, the coating having enough flexibility so that it will not crack or chip off.

If the wire is not to be used at once, preferably it should receive a collodion coating so as to 60 avoid moisture absorption by the coating. This coating may best be applied by placing the wire in a vessel containing a solution of collodion and allowing the wire to remain in this solution until the occluded gas escapes, being displaced by the 65 collodion which then forms an adherent skin layer. Water absorption may also be avoided by subjecting the coating to a high temperature so as to vitrify the material thereof, and should be used preferably only when the filament is formed 70 prior to heating.

When properly placed in a lamp, the lamp may be exhausted in the ordinary manner. To do this it is necessary to raise the temperature of the filament a great deal higher than it is heated in 75 normal operation, the temperature in some in-

stances reaching as high as 2,000° C. At this temperature the first or inner layer of beryllium aluminosilicate will fuse with the resistance wire and form a dense, hard, flexible coating which is substantially integral with the wire. The beryllium oxide, however, which forms the outer layer or surface of the insulating filament, will withstand temperatures in the neighborhood of 2400° C. without melting, and therefore is not affected by the high temperature used in exhausting the lamp. At the exhausting temperature, all physically or chemically unstable components of the coating are discharged so that the resistance wire and coating may be completely degasified. There is, however, a slight chemical action between the inner and outer layers which firmly knits the two together, thus making a substantially integral structure.

While beryllium oxide has highly desirable characteristics, as an external coating, and is used as a preferred material, I have found that aluminum oxide might be used with the beryllium oxide or even be used alone, although this material does not have all the desirable properties of beryllium oxide for lamp filament use.

As indicated above, still other materials may be used as an insulating coating, and I do not, therefore, desire to limit the invention to any specific material, except as defined in the claims hereto appended.

What I claim is:

1. In a lamp construction the combination of an element, a base therefor, filament supporting means mounted within the envelope and on said base, and a filament mounted on the filament support, said filament consisting of a refractory base element, and a coating thereon formed of an insulating compound of a metal having low atomic number, and an outer coating of another insulating compound of a metal having low atomic number.

2. In a lamp construction the combination of an envelope, a base therefor, filament supporting means mounted within the envelope and on said base, and a filament mounted on the supporting means, said filament consisting of a refractory metal core, a layer of an insulating metallic silicate fused to the surface of the core, and an insulating oxide in close contact with said silicate.

3. In a lamp construction the combination of an envelope, a base therefor, filament supporting means mounted in the envelope and on said base, and a filament mounted on the support, said filament consisting of a refractory metal base, a coating of beryllium aluminosilicate fused to said base, and a coating of beryllium oxide closely associated with said fused coating.

4. In a lamp construction the combination of an envelope, a base therefor, filament supporting means mounted in the envelope and on said base, and a filament mounted on the support, said filament consisting of a refractory metal base, a coating of an insulating metallic silicate and a binder on said base, and an outer insulating coating of an oxide and a binder.

5. In a lamp construction the combination of an envelope, a base therefor, filament supporting means mounted in the envelope and on said base, and a filament mounted on the support, said filament consisting of a refractory metal base, a coating of beryllium aluminosilicate mixed with the solution of ammonium borate on said base, and an outer coating of beryllium oxide mixed with the solution of ammonium borate on said first coating.

SAMUEL RUBEN. 100